# EUROPEAN PATENT APPLICATION

(11) **EP 0 889 485 A1**
(43) Date of publication of application: **07.01.1999**
(21) Application number: 96942664.2
(22) Date of filing: 27.12.1996
(51) Int. Cl.: H01B 3/52

(54) **OIL-IMPREGNATED INSULATING PLASTIC LAMINATED PAPER, KRAFT PAPER FOR USE IN LAMINATED PAPER AND POWER CABLE USING THE SAME**

(71) Applicant: Fujikura, Ltd., Tokyo 135-0042 (JP)
(72) Inventor: TAKAHASHI, Tohru, Tokyo 136 (JP); MIYATA, Hiroyuki, Chiba 275 (JP); IINUMA, Kohichi, Koto-ku Tokyo 135 (JP); YOSHIDA, Shotaro, Tokyo 132 (JP); SHIGETOSHI, Ikuo, Chiba 285 (JP)
(74) Representative: Picard, Jean-Claude Georges
(86) International application number: JP9603853
(87) International publication number: WO9829878

(57) **Abstract**

This invention relates to an plastic laminated paper used for an oil-impregnated insulator in an OF cable and the like, a kraft paper used in the laminated paper and an electrical cable using the laminated paper. The objects of this invention is to increase the adhesion strength between the kraft paper and a plastic film of the laminated paper comprising kraft paper and the plastic film, and to improve the impulse dielectric breakdown character of the oil-impregnated insulator obtained by using this laminated paper.

The present invention adopts a multi-ply paper comprising at least two layers of paper having different air permeability as the kraft paper for solving the objects. The air permeability of the high air permeability layer is set to be equal to or less than 5000 Gurley seconds, and the air permeability of the low air permeability layer is set to be equal to or greater than 1000 Gurley seconds.

## Description

### Field of the Invention

The present invention relates to a plastic laminated paper for oil-impregnation insulation and used in an oil-impregnated insulator of an electrical cable such as an OF cable, a kraft paper used in the laminated paper and the electrical cable in which it is used. The present invention increases in particular the adhesion strength of the kraft paper and a plastic film and improves the impulse breakdown character of the oil-impregnated insulator in which these are used.

Additionally, this electrical cable is suitable for direct and alternating current transmission.

### Description of the Related Art

As a plastic laminated paper forming an oil-impregnated insulator in an OF cable, at present, a polypropylene laminated paper wherein kraft papers are stuck to both surfaces of a polypropylene film is widely used. This is because this polypropylene laminated paper has superior dielectric and breakdown character compared to conventional kraft paper.

The fabrication method of the plastic laminated paper, such as the polypropylene laminated paper, begins with extrusion of a melted plastic film from a T-die of an extruder. While in a melted state, both surfaces of this film are paralleled with kraft paper. After the adhesion by roller pressure, it is cooled and wound.

Therefore, the plastic film and the kraft paper of the plastic laminated paper simply adhere to each other by the anchoring effect caused by the penetration of melted plastic into the fine roughness on the surface of the kraft paper, and generally the adhesion strength between the plastic film and the kraft paper is weak.

In order to increase the adhesion strength, providing the adhesive on the interface between the plastic film and the kraft paper has been proposed. However, the use of the adhesive is prohibited because it causes the deterioration of dielectric character since the adhesive is generally a substance which has polar radicals.

Accordingly, any means is necessary to increase the adhesion strength between the plastic film and the kraft paper without using the adhesive.

Increasing the adhesion strength by boost of the anchor effect has been considered as one of the means, and in order to implement this the use of a kraft paper having high air permeability has been considered effective. Because the surface of the high air permeability kraft paper has large roughness, the degree of penetration of resin laminated onto the paper becomes high. Therefore, the anchor effect is boosted, and the adhesion strength is also increased.

However, the plastic laminated paper made of the high air permeability kraft paper has a disadvantage that the dielectric breakdown character, in particular the impulse breakdown voltage, of the oil-impregnated insulator obtained from this plastic laminated paper deteriorates.

Additionally, the oil-impregnated insulator comprising the plastic laminated paper is used in the oil-impregnated state. In such oil-impregnated state, the adhesion strength between the kraft paper and the plastic film is further remarkably weakened because of swelling of the plastic film due to oil absorption. When the temperature rises, in particular during the laying of OF cable, the adhesion strength decreases furthermore.

### Disclosure of the Invention

In consideration of the above problems, it is the object of the present invention to sufficiently increase the adhesion strength between the plastic film and the kraft paper of the plastic laminated paper which forms an oil-impregnated insulator such as an OF cable, and to increase the insulation breakdown character of the oil-impregnated insulator made of the plastic laminated paper.

The kraft paper for the plastic laminated paper of the present invention is a multi-ply paper comprising at least two layers of paper having different air permeability. The air permeability of the low air permeability layer of this kraft paper is equal to or greater than 1000 Gurley seconds, preferably equal to or greater than 2000 Gurley seconds, on the other hand, the air permeability of the high air permeability layer of this kraft paper is equal to or less than 5000 Gurley seconds, preferably equal to or less than 2000 Gurley seconds, and even more preferably equal to or less than 20 Gurley seconds.

In addition, the low air permeability layer can be a high density layer, having the density exceeding 0.7 g/cm³, and the high air permeability layer can be a low density layer, having the density equal to or less than 0.7 g/cm³. It is desirable that the high density and low air permeability layer is a fourdrinier paper, and the low density and high air permeability layer is a cylindrical paper.

Further, it is preferable that the thickness of the low air permeability layer is at least 15 µm, and the thickness of the high air permeability layer is at least 5 µm.

Furthermore, said multi-ply kraft paper is converted into the plastic laminated paper of the present invention by sticking the high air permeability layer of said multi-layer kraft paper onto a plastic film.

Incidentally, among the plastic film, polypropylene film is preferable, and it is desirable that the polypropylene is homopolymer having the melt index of 5 ∼ 50 g / 10 minutes.

Finally, the electrical cable of the present invention has an oil-impregnated insulator which is made by the wind of the plastic laminated paper and the oil-impregnation.

### Brief Description of the Drawings

Fig. 1 is a generalized cross-section figure showing a first example of the kraft paper of the present invention.
Fig. 2 is a generalized cross-section figure showing a second example of the kraft paper of the present invention.
Fig. 3 is a generalized cross-section figure showing a third example of the kraft paper of the present invention.

### Preferred Embodiments of the Present Invention

### (1) Kraft Paper

Fig. 1 shows a first example of the kraft paper of the present invention, and this example is a two-ply kraft paper comprising two layers 1a, 1b having different air permeability.

The first layer 1a is a high air permeability layer, and the second layer 1b is a layer having the air permeability lower than that of the first high air permeability layer 1a. The air permeability of the first high air permeability layer 1a is equal to or less than 5000 Gurley seconds, preferably equal to or less than 2000 Gurley seconds, and further preferably equal to or less than 20 Gurley seconds because the air permeability exceeding 5000 Gurley seconds gives the disadvantage such as the deterioration of adhesiveness with a plastic film.

On the other hand, the air permeability of the second low air permeability layer 1b is equal to or greater than 1000 Gurley seconds, preferably equal to or greater than 2000 Gurley seconds, and even more preferably equal to or greater than 4000 Gurley seconds because the air permeability less than 1000 Gurley seconds gives the disadvantage that the impulse breakdown voltage falls if the kraft paper is used in an oil-impregnated insulator.

Additionally, the thickness of this two-ply kraft paper 1 is not limited in particular, but typically, it is in the range of 20 ∼ 100 µm. The thickness of the high air permeability layer is at least 5 µm, and preferably in the range of 5 ∼ 30 µm. In contrast, the thickness of the low air permeability layer is at least 15 µm, and preferably in the range of 15 ∼ 17 µm. If the thickness of the first layer 1a is less than 5 µm, the adhesion strength with the plastic film becomes insufficient, and if the thickness of the second layer 1b is less than 15 µm, the impulse breakdown voltage deteriorates.

Furthermore, with regard to each ratio of the thickness of the high air permeability layer 1a and the low air permeability layer 1b to the total thickness of the two-ply kraft paper 1, it is advantageous that the ratio of the high air permeability layer 1a is smaller than that of the low air permeability layer. This is because the area contributing to the adhesiveness is a relatively thin part under the surface, and if the roughness of the surface are large, sufficient adhesive strength can be attained. Further, this is because the thicker the low air permeability layer 1b becomes, the more the impulse breakdown character is improved.

In addition, as the above two-ply kraft paper 1, a low loss paper bathed in deionized water which has good dielectric character is preferable, and a low conductive paper having the conductivity of aqueous extract equal to or less than 15 µS / cm (conforming to JIS-C-2111) is preferable.

Such the two-ply kraft paper 1 is manufactured by the way such as piling the fibrillized pulp of the paper fiber on top of the other in a dry or wet process using a fourdrinier or cylinder paper machine.

Fig. 2 shows the second example of the kraft paper of the present invention.

This kraft paper 11 is a three-ply kraft paper. This three-ply kraft paper 11 comprises the high air permeability layer constituting the outer surfaces 11a and 11a and the low air permeability layer 11b therebetween.

Additionally, the air permeability of the high air permeability layer of the outer surfaces 11a and 11a are equal to or less than 5000 Gurley seconds, preferably equal to or less than 2000 Gurley seconds and more preferably between 20 ∼ 5000 Gurley seconds, and the air permeability of the low air permeability layer of the inner part 11b is equal to or greater than 1000 Gurley seconds, preferably equal to or greater than 4000 Gurley seconds and more preferably between 4000 ∼ 2000 Gurley seconds.

The thickness of this three-ply kraft paper 11 is not limited in particular, but is typically in a range of 20 ∼ 100 µm.

Furthermore, with regard to each ratio of the thickness of the high air permeability layer 11a and the low air permeability layer 11b to the total thickness of the three-ply kraft paper 11, it is advantageous that the ratio of the high air permeability layer 11a is smaller than that of the low air permeability layer. This is because the area contributing to the adhesiveness is a relatively thin part under the surface, and if the roughness of the surface are large, sufficient adhesive strength can be attained. Further, this is because the thicker the low air permeability layer 11b becomes, the more the impulse breakdown character is improved.

Typically, the thickness of the high air permeability layer 11a is at least 5 µm, preferably between 5 ∼ 20 µm, and the thickness of the low air permeability layer 11b is at least 15 µm, preferably between 15 ∼ 60 µm.

Additionally, the use of a low loss paper bathed in deionized water, which has good dielectric character, is also preferable for the three-ply kraft paper 11.

Fig. 3 shows the third example of the kraft paper of the present invention.

This kraft paper 21 is a two-ply kraft paper. The first layer 21a is a high air permeability layer and the second layer 21b is a low air permeability layer. The density of the first high air permeability layer 21a is equal to or less than 0.7 g / cm³, preferably equal to or less than 0.6 g / cm³, more preferably in the range of 0.6 ∼ 0.5 g / cm³. If the density exceeds 0.7 g / cm³, the adhesiveness with the plastic film deteriorates and this becomes disadvantage. Additionally, the first high air permeability layer 21a is also a high air permeability layer which has the air permeability equal to or less than 2000 Gurley seconds, preferably equal to or less than 20 Gurley seconds.

In addition, the air permeability of the second low air permeability layer 21b is equal to or greater than 10000 Gurley seconds, preferably equal to or greater than 30000 Gurley seconds. If the air permeability is less than 10000 Gurley seconds, the impulse breakdown voltage deteriorates if it is used in an oil-impregnated insulator.

Additionally, the second low air permeability layer 21b is also a high density layer which has the density over 0.7 g / cm³, preferably over 0.9 g / cm³.

Furthermore, in this example, it is preferable that the first high air permeability and low density layer 21a is a cylindrical paper manufactured by using a cylinder paper machine in a wet process, and that the second low air permeability and high density layer 21b is a fourdrinier paper manufactured by using a fourdrinier paper machine in a wet process. Then, in the above case, the ratio of the thickness of the second and fourdrinier paper layer 21b to the first and cylindrical paper layer 21a is set about between 0.8 ∼ 3.

The kraft paper of this example is laminated so that a plastic film and the first low density and high air permeability layer 21a are in contact with each other, and after the plastic laminated paper is made, it is cut into tapes, and the tape is wound. In these procedures, there is no breakage of the kraft paper when cutting is done, it is easy to wind, and further there is little difference between the vertical and the horizontal direction with regard to the tensile strength, stretching, Young's modulus and so on. Further, the kraft paper is not anisotropic but homogeneous, and has good adhesiveness with a plastic film. And, good impulse breakdown strength is expected if the kraft paper is used in an oil-impregnated insulator.

The kraft paper of the present invention can be a multi-ply kraft paper in which the high air permeability and the low air permeability layers are piled up over three layers. In this case, at least one of the layers which is in contact with a plastic film should be the high air permeability layer having the air permeability equal to or less than 5000 Gurley seconds, preferably equal to or less than 2000 Gurley seconds, and more preferably 20 Gurley seconds. On the other hand, the other layers should have the air permeability equal to or greater than 1000 Gurley seconds, preferably equal to or greater than 2000 Gurley seconds, and more preferably equal to or greater than 4000 Gurley seconds, which is selected so that their air permeability is lower than that of the high air permeability layer.

### (2) The plastic laminated paper

The plastic laminated paper of the present invention is the lamination of the above-described kraft paper and a plastic film. This laminating is carried out by the extrusion lamination method wherein a melted plastic film is extruded from a T-die of an extruder, and while the film is in a melted state, both or either surface of the film is paralleled with the kraft paper and put together by pressure rolls.

When laminating, no matter which kind of the above kraft paper is used, the high air permeability layer is always set to be in contact with the plastic film. In the case of laminating the three-ply kraft paper 11 described in the second example, the check of the surface of the kraft paper is not necessary because both the outer surfaces 11a and 11a are high air permeability layers. In the case of laminating the two-ply kraft paper 21 described in the third example, the first, low density and high air permeability layer 21a is set to be in contact with the plastic film.

The plastic film with thickness of 20 ∼ 150 µm made from non-polar polyolefins such as polypropylene, poly-4-methylpentene-1, polybutene-1, polyethylene and so on, and fluorocarbon resin such as tetrafluoroethylene-hexafluoropropylene copolymer, ethylene-tetrafluoroethylene copolymer and so on, is used as the above plastic film. Among these plastics, a film of polypropylene homopolymers, preferably a film made from polypropylene homopolymer having comparative low melt viscosity such that melt index is between 5 ∼ 50 g / minute, is desirable because it has high adhesiveness with the kraft paper, and good insulation character of the laminated paper which is obtained from the film is expected.

It the melt index of the polypropylene is less than 5, the melt viscosity at the time of extruding the melted polypropylene becomes large. Therefore, it becomes difficult for the resin to penetrate into the roughness of the surface of kraft paper, and the adhesive strength between the polypropylene film and the kraft paper deteriorates. If melt index exceeds 50, the melt viscosity becomes too small. Therefore, the back pressure at the time of extruding becomes unstable and the fluctuation of the thickness of the laminated paper becomes large.

Additionally, polypropylene homopolymer have superior swelling character against insulation oil compared to copolymers such as random and block copolymer.

The thickness of the plastic laminated paper which is mentioned above is in the range of 100 ∼ 300 µm. However, depending on the use and so on, it is not necessary to keep it within this range.

In the case of plastic laminated paper having such structures mentioned above, the adhesive strength becomes high because the melted plastic is easy to penetrate into the kraft paper, wherein the contacting layer to be laminated onto the plastic film is porous and has big roughness due to the low density of the layer. And, the impulse breakdown strength when this plastic laminated paper is used in an oil-impregnated insulator becomes high because most of the other layers of the kraft paper are the high density layers.

### (3) Electrical Cable

The electrical cable of the present invention is made by impregnation of insulation oil such as polybutene and alkylbenzene oil into the insulator covered with a shielding layer, sheath, anti-corrosive layer and so on. The insulator is made by the large number of wind of said plastic laminated paper onto a conductor directly or indirectly via a shielding layer.

If low viscous oil is used as the insulation oil and the oil is under the constant pressure greater than air pressure, an OF cable is obtained.

In addition, if high viscous oil such that its kinetic viscosity is equal to or greater than 500 centistokes at 30 °C is used as the insulation oil, MIND (Mass Impregnated Non-Draining) cable which is preferable for a long distance undersea cable, wherein the insulation oil cannot be pressurized, is obtained.

In this electrical cable, the insulation character, in particular the impulse breakdown strength, is good and the plastic laminated paper does not separate into the kraft paper and the plastic film when treating the cable, in which the insulator is exposed, at the time of connecting the cable.

The electrical cable of the present invention is suitable as a direct current cable or an alternating current cable in OF cable for transmission of extra/ultra high voltage.

Hereunder, we specify the function and effect of the present invention referring specific examples, however, the present invention should not be restricted to these examples.

### Experimental Example 1

Polypropylene homopolymer with the melt index of 15.0 g / minute (JIS K6758) and the density of 0.90 g / cm³ was melted and extruded at 280°C for making a polypropylene film, and while in the melted state, both of the film surfaces were lined with the kraft paper having the density of 0.75 g / cm³ and the thickness of 40 µm, and they were stuck together by pressure rolls to make a polypropylene laminated paper with the total thickness of 170 µm.

As the kraft paper, a normal single layer paper or a two-ply paper, which was made from two layers having different air permeability and thickness of 20 µm, were used.

In the case of the two-ply kraft paper, the high air permeability side was faced to the polypropylene film surface and the low air permeability side constituted the outer surface.

The adhesion strength (180° exfoliation test) at the interface between the polypropylene film and the kraft paper of each polypropylene laminated paper, wherein the kraft paper was variously changed in terms of the air permeability, was measured. Each polypropylene laminated paper was wound around a conductor to form an oil-impregnated insulator having the thickness of about 1 mm (JIS-C-2320, Type 2, Number 1 alkyl benzene oil was impregnated), and to form a model cable finally. Each of the positive polarity impulse breakdown voltage of the model cable was measured. The results are shown in Fig. 1.

| Fig. 1 | | | | |
|---|---|---|---|---|
| Experiment Number | Kraft Paper | | Adhesion Strength (g /15 mm width) | Impulse Breakdown Voltage (kv /mm) |
| | Number of Layers | Air Permeability (Gurley seconds) | | |
| 1 - 1 | One-ply (40 µm) | 100 | 500 | 100 |
| 1 - 2 | | 5000 | 150 | 130 |
| 1 - 3 | | 7000 | 20 | 140 |
| 1 - 4 | two-ply (20 µm x 2) | High layer side 100 | 500 | 105 |
| | | Low layer side 500 | | |
| 1 - 5 | | High layer side 100 | 500 | 125 |
| | | Low layer side 1000 | | |
| 1 - 6 | | High layer side 100 | 500 | 145 |
| | | Low layer side 20000 | | |
| 1 - 7 | | High layer side 5000 | 150 | 145 |
| | | Low layer side 20000 | | |
| 1 - 8 | | High layer side 7000 | 20 | 145 |
| | | Low layer side 20000 | | |

### Experimental Example 2

Polypropylene homopolymer with the melt index of 15.0 g / minute (JIS K6758) and the density of 0.90 g / cm³ was melted and extruded at 280°C for making a polypropylene film, and while in the melted state, both of the film surfaces were lined with the two-ply kraft paper having the thickness of 40 µm, and they were stuck together by pressure rolls to make a polypropylene laminated paper with the total thickness of 170 µm.

As the two-ply kraft paper, a kraft paper having a high air permeability layer with thickness of 15 µm and a low air permeability layer with thickness of 25 µm, and having the conductivity of aqueous extract of 5 µS / cm according to JIS-C-2111, was used. The high air permeability layer was faced to the polypropylene film surface and the low air permeability layer constituted the outer surface.

The adhesion strength (180° exfoliation test) at the interface between the polypropylene film and the two-ply kraft paper of each polypropylene laminated paper alter the impregnation with alkyl benzene oil at 100 °C (JIS-C-2320, Type 2, Number 1) for 24 hours was measured. Each polypropylene laminated paper was wound around a conductor to form an oil-impregnated insulator having the thickness of about 1 mm (JIS-C-2320, Type 2, Number 1 oil was impregnated), and to form a model cable finally. Each of the positive polarity impulse breakdown voltage of the model cable was measured. The results are shown in Fig. 2

| Fig. 2 | | | | |
|---|---|---|---|---|
| Experiment Number | Two-ply Kraft Paper Air Permeability (Gurley seconds) | | Adhesion Strength with Impregnated Heated Oil (g / 15 mm) | Impulse Breakdown Voltage (kV / mm) |
| | High Air Permeability Layer | Low Air Permeability Layer | | |
| 2 - 1 | 50 | 10000 | 50 | 140 |
| 2 - 2 | 15 | 10000 | 400 | 140 |
| 2 - 3 | Equal to or less than 5 | 10000 | 500 | 140 |
| 2 - 4 | Equal to or less than 5 | 4500 | 500 | 135 |
| 2 - 5 | Equal to or less than 5 | 3000 | 500 | 110 |

### Experimental Example 3

Polypropylene homopolymer with the melt index of 15.0 g / minute (JIS K6758) and the density of 0.90 g / cm³ was melted and extruded at 280°C for making a propylene film, and while in the melted state, both of the film surfaces were lined with the kraft paper having the density of 0.75 g / cm³ and the thickness of 40 µm, and they were stuck together by pressure rolls to make a polypropylene laminated paper with the total thickness of 170 µm.

As the kraft paper, a normal single layer paper or a two-ply paper which was made from layers having different thickness, and in which the air permeability of the high air permeability layer was equal to or less than 20 Gurley seconds and the air permeability of the low air permeability layer was equal to or greater than 20000 Gurley seconds, was used. In the case of the two-ply kraft paper, the high air permeability layer was faced to the polypropylene film surface and the low air permeability layer constituted the outer surface.

The adhesion strength (180° exfoliation test) at the interface between the polypropylene and the kraft paper of each obtained polypropylene laminated paper was measured.

Additionally, each polypropylene laminated paper was wound around a conductor to form an oil-impregnated insulator having the thickness of about 1 mm (JIS-C-2320, Type 2, Number 1 alkyl benzene oil was impregnated), and to form a model cable finally. Each of the positive polarity impulse breakdown voltage of the model cable was measured. The results are shown in Fig. 3.

| Fig. 3 | | | | |
|---|---|---|---|---|
| Experiment Number | Two-ply Kraft Paper Thickness (µm ) | | Adhesion Strength (g / 15 mm) | Impulse Breakdown Voltage (kV / mm) |
| | High Air Permeability Layer(µm ) | Low Air Permeability Layer(µm ) | | |
| 3 - 1 | 0 | 40 | 15 | 145 |
| 3 - 2 | 3 | 37 | 30 | 145 |
| 3 - 3 | 5 | 35 | 150 | 145 |
| 3 - 4 | 10 | 30 | 200 | 140 |
| 3 - 5 | 15 | 25 | 450 | 140 |
| 3 - 6 | 25 | 15 | 500 | 135 |
| 3 - 7 | 30 | 10 | 500 | 105 |

### Experimental Example 4

A polypropylene laminated paper was manufactured, and the adhesion strength and the positive polarity impulse breakdown voltage was measured like in Experimental Example 3 except that the kraft paper, wherein the thickness of the high air permeability layer was set to be 15 µm and the thickness of the low air permeability layer was set to be 25 µm, and the air permeability of each layer was changed, was used as the two-ply paper. The results are shown in Fig. 4.

| Fig. 4 | | | | |
|---|---|---|---|---|
| Experiment Number | Two-ply Kraft Paper Air Permeability (Gurley seconds) | | Adhesion Strength (g / 15 mm) | Impulse Breakdown Voltage (kV / mm) |
| | High Air Permeability Layer | Low Air Permeability Layer | | |
| 4 - 1 | 2000 | Equal to or greater than 20000 | 200 | 140 |
| 4 - 2 | 3000 | Equal to or greater than 20000 | 80 | 140 |
| 4 - 3 | equal to or less than 20 | 4000 | 500 | 135 |
| 4 - 4 | equal to or less than 20 | 2000 | 500 | 110 |

### Experimental Example 5

Polypropylene homopolymer with the melt index of 15.0 g / minute (JIS K6758) and the density of 0.90 g / cm³ was melted and extruded at 280° C for making a polypropylene film, and while in the melted state, both of the film surfaces were lined with the kraft paper having the density 0.75 g / cm³ and the thickness of 40 µm, and they were stuck together by pressure rolls to make a polypropylene laminated paper with the total thickness of 170 µm.

As the kraft paper, a three-ply paper having the total thickness of 45 µm, which was made by sticking two sheets of the high air permeability paper having thickness of 15 µm on both surfaces of a low air permeability paper having the thickness of 15 µm and the density of 0.75 g / cm³, was used.

Either high air permeability surface of the three-ply kraft paper was faced to the polypropylene film surface.

The adhesion strength (180° exfoliation test) at the interface between the polypropylene film and the kraft paper of each polypropylene laminated paper, wherein the kraft paper was variously changed in terms of the air permeability, was measured. Additionally, each polypropylene laminated paper was wound around a conductor to form an oil-impregnated insulator having the thickness of about 1 mm (JIS-C-2320, Type 2, Number 1 alkyl benzene oil was impregnated), and to form a model cable finally. Each of the positive polarity impulse breakdown voltage was measured. The results are shown in Fig. 5.

| Fig. 5 | | | | |
|---|---|---|---|---|
| Experiment Number | Kraft Paper | | Adhesiong Strength (g/ 15 mm width) | Impulse Breakdown Voltage (kv / mm) |
| | Number of Layers | Air Permeability (Gurley seconds) | | |
| 5 - 1 | Three-ply (15 µm x 3) | High layer side 100 | 500 | 105 |
| | | Low layer side 500 | | |
| | | High layer side 100 | | |
| 5-2 | | High layer side 100 | 500 | 125 |
| | | Low layer side 1000 | | |
| | | High layer side 100 | | |
| 5 - 3 | | High layer side 100 | 500 | 145 |
| | | Low layer side 20000 | | |
| | | High layer side 100 | | |
| 5 - 4 | | High layer side 5000 | 150 | 145 |
| | | Low layer side 20000 | | |
| | | High layer side 5000 | | |
| 5 - 5 | | High layer side 7000 | 20 | 145 |
| | | Low layer side 20000 | | |
| | | High layer side 7000 | | |

### Experimental Example 6

Polypropylene homopolymer with the melt index of 15.0 g / minute (JIS K6758) and the density of 0.90 g / cm³ was melted and extruded at 280°C for making a propylene film, and while in the melted state, both of the film surfaces were lined with the two-ply kraft paper having the thickness of 40 µm and different layers in terms of the air permeability and the density, and they were stuck together by pressure rolls to make a polypropylene laminated paper with the total thickness of 170 µm.

As the two-ply kraft paper, a kraft paper having a low density layer with thickness of 15 µm and a low air permeability layer with thickness of 25 µm, and having the conductivity of aqueous extract of 5 µS / cm according to JIS-C-2111, was used. The low density layer was faced to the polypropylene film surface and the low air permeability layer constituted the outer surface. The density of the low density layer and the air permeability of the low air permeability layer were changed.

The adhesion strength (180° exfoliation test) at the interface between the polypropylene film and the two-ply kraft paper of each polypropylene laminated paper after the impregnation with alkyl benzene oil at 100 °C (JIS-C-2320, Type 2, Number 1) for 24 hours was measured. Each polypropylene laminated paper was wound around a conductor to form an oil-impregnated insulator having the thickness of about 1 mm (JIS-C-2320, Type 2, Number 1 oil was impregnated), and to form a model cable finally. Each of the positive polarity impulse breakdown voltage of the model cable was measured. The results are shown in Fig. 6

| Fig. 6 | | | | |
|---|---|---|---|---|
| Experiment Number | Density and Air Permeability of Two-ply Kraft Paper | | Adhesion Strength with Impregnated Heated Oil (g / 15 mm width) | Impulse Breakdown Voltage (kV / mm) |
| | Low Density Layer (g/cm³) | Low Air Permeability Layer (Gurley seconds) | | |
| 6 - 1 | 0.69 | 20000 | 400 | 135 |
| 6 - 2 | 0.75 | 20000 | 50 | 135 |
| 6 - 3 | 0.58 | 30000 | 500 | 140 |
| 6 - 4 | 0.72 | 5000 | 150 | 110 |
| 6 - 5 | 0.58 | 5000 | 500 | 110 |

### Experimental Example 7

The various polypropylene homopolymer with the density of 0.90 g / cm³ and the melt index between 2 ∼ 70 g / 10 minutes (JIS K6758) was melted and extruded at 280° C for making a polypropylene film, and while in the melted state, both of the film surfaces were lined with two-ply kraft paper, and they were stuck together by pressure rolls to produce a polypropylene laminated paper with the total thickness of 170 µm.

As the two-ply kraft paper, the kraft paper consisted of a high air permeability layer (thickness of 10 µm), of which the air permeability is equal to or less than 20 Gurley seconds, and of a low air permeability layer (thickness of 30 µm), of which the air permeability is equal to or greater than 10000 Gurley seconds, was used. And, the high air permeability layer was stuck onto the polypropylene film. The adhesion strength (180° exfoliation test) at the interface between the polypropylene film and the kraft paper of the obtained polypropylene laminated paper was measured. The results are shown in Fig. 7

| Fig. 7 | | | |
|---|---|---|---|
| Experiment Number | Melt Index of Polypropylene (g / 10 min) | Adhesion Strength | Comments |
| 7 - 1 | 5 | 350 | |
| 7 - 2 | 15 | 500 | |
| 7 - 3 | 50 | 500 | |
| 7 - 4 | 70 | 500 | large thickness fluctuation |
| 7 - 5 | 2 | 50 | |

### Industrial Use

The OF cable in which the plastic laminated paper of the present invention is used has superior impulse breakdown character specially, and can be used as a high voltage or extra/ultra high voltage direct and alternating current transmission cable. In addition, because the adhesion strength between the kraft paper and the laminated paper is high, they are not separated even if the laminated paper tape is wound or the cable is connected to another, for example, and there is no deterioration of the operationality.

## Claims

1. A kraft paper used for a plastic laminated paper characterized in that the kraft paper which is laminated onto a melted extruded plastic film of the plastic laminated paper for oil-impregnation insulation is a multi-ply paper comprising at least two layers of paper having different air permeability.

2. A kraft paper used for a plastic laminated paper characterized in that the kraft paper which is laminated onto a melted extruded plastic film of the plastic laminated paper for oil-impregnated insulation is a multi-ply paper comprising at least two layers of paper having different air permeability, wherein the thickness of the high air permeability layer is at least 5 µm and the thickness of the low air permeability layer is at least 15 µm.

3. A kraft paper used for a plastic laminated paper according to Claim 1 and 2, wherein the air permeability of the high air permeability layer is equal to or less than 5000 Gurley seconds and the air permeability of the low air permeability layer is equal to or greater than 1000 Gurley seconds.

4. A kraft paper used for a plastic laminated paper according to Claim 3, wherein the air permeability of the high air permeability layer is equal to or less than 2000 Gurley seconds and the air permeability of the low air permeability layer is equal to or greater than 2000 Gurley seconds.

5. A kraft paper used for a plastic laminated paper according to Claim 4, wherein the air permeability of the high air permeability layer is equal to or less than 20 Gurley seconds and the air permeability of the low air permeability layer is equal to or greater than 4000 Gurley seconds.

6. A kraft paper used for a plastic laminated paper characterized in that the kraft paper which is laminated onto a melted extruded plastic film of the plastic laminated paper for oil-impregnation insulation is a multi-ply paper comprising at least three layers of paper having different air permeability, wherein both outer surfaces of said multi-ply paper consist of high air permeability layers and the inner part consist of a low air permeability layer.

7. A kraft paper used for a plastic laminated paper according to Claim 6, wherein the air permeability of both the outer surface layers of said multi-ply paper is equal to or less than 5000 Gurley seconds and the air permeability of the inner part layer is equal to or greater than 1000 Gurley seconds.

8. A kraft paper used for a plastic laminated paper characterized in that the kraft paper which is laminated onto a melted extruded plastic film of the plastic laminated paper for oil-impregnation insulation is a multi-ply paper comprising a low density layer having density equal to or less than 0.7 g / cm³ and a low air permeability layer having the air permeability equal to or greater than 10000 Gurley seconds.

9. A kraft paper used for a plastic laminated paper characterized in that the kraft paper which is laminated onto a melted extruded plastic film of the plastic laminated paper for oil-impregnation insulation is a multi-ply paper comprising at least two layers of paper having different air permeability, wherein the low air permeability layer is a fourdrinier paper and the high air permeability layer is a cylindrical paper.

10. A plastic laminated paper for oil-impregnation insulation characterized in that the kraft paper in any one of Claim 1 to 9 used for the plastic laminated paper is laminated onto a melted extruded plastic film so that the high air permeability layer of the kraft paper is in contact with the plastic film surface.

11. A plastic laminated paper for oil-impregnation insulation according to Claim 10, wherein said melted extruded plastic film is a polypropylene film.

12. A plastic laminated paper for oil-impregnation insulation according to Claim 11, wherein said polypropylene film is made from polypropylene homopolymer having the melt index of 5 ∼ 50 g / 10 minutes.

13. An electrical cable characterized in using the plastic laminated paper for oil-impregnation insulation in any one of Claims 10 to 12 as an oil-impregnated insulator.
